

# United States Patent Office

2,759,834

Patented Aug. 21, 1956

1

2,759,834

## REFRACTORY AND PROCESS FOR MAKING SAME

Himansu Kumar Mitra, Jamshedpur, Bihar, India

No Drawing. Application April 22, 1953,  
Serial No. 350,516

1 Claim. (Cl. 106—59)

This invention relates to a process for manufacturing a refractory material of the neutral and neutral-to-basic type from a low grade, high silicious, non-refractory chrome ore, and the article formed thereby. The refractory produced by the method of this invention possesses superior physical properties, e. g., high refractoriness-under-load and high resistance against attack of iron oxide. The present application is a continuation-in-part of co-pending application Serial No. 74,863 filed February 5, 1949 now abandoned.

In the past the production of a high grade refractory material has been limited to the use of chrome ore characterized by a high pyrometric cone equivalent (fusion point), e. g., above cone 35 (above 1785° C.), and which did not contain more than 10% silica.

Thus, Parmellee and Ally [Parmellee C. W. and Ally A. "Some Properties of Chrome Spinel," J. Am. Ceram. Soc. 15 (4) 213 (1932)] quoting McDowell state that for chrome brick manufacture,  $\text{SiO}_2$  content of up to 5% in the chrome ore is allowed; from 5 to 9% is generally penalized and above 9% is rejected.

Litinsky [Litinsky L. "Recent Development in the Production of Refractories Containing Magnesia," Iron & Steel Industry p. 498 Sept. (1936)] states that for chrome-magnesite brick the chrome ore employed should contain as much  $\text{Cr}_2\text{O}_3$  and as little  $\text{SiO}_2$  as possible.

U. S. Patent No. 2,077,796 of April, 1937, for making chrome-magnesite brick gives the silica content of refractory grade chrome ore used, as 4.5%.

Schauer [Schauer T. "Evaluation of Chrome Ores for the Manufacture of Refractories" Tonid-Ztg. 63 (61) 701-702 I (62) 724-725 (1939)] states too much  $\text{SiO}_2$  in chrome ore decreases refractoriness-under-load. In evaluating chrome ore for the manufacture of refractories he suggests that if the quotient for the equation:

$$\frac{\text{Percent MgO}}{\text{Percent Al}_2\text{O}_3} \quad 2.67$$

$$\text{Percent SiO}_2$$

is less than 1.38, it indicates lowered refractoriness, and resistance to temperature changes.

The use of low grade chrome ores which do not conform to the aforesaid specifications has also been attempted by first physically treating such ores to reduce the silica content to less than 10%. When successful, the beneficiation of such ores, e. g., by physical means such as washing, had the effect of producing an ore that would conform to the aforesaid specification. This treated ore was then employed in a conventional process of manufacture of high grade refractory.

It is obvious that in this known method of beneficiation, not only an extra process step was involved, but it also resulted in a loss of some of the material which otherwise could be turned into a valuable refractory material.

The attempted use of low grade chrome ores did not always meet with success as in some cases it was not possible to reduce the silica content to less than 10% solely by physically treating. These chrome ores have

2

always been avoided as a source of refractory material for this reason.

It is, accordingly, an object of this invention to employ a low-grade non-refractory, highly silicious, hybrid chrome ore for the manufacture of a superior grade of refractory, without subjecting the raw material to any process of beneficiation.

So far as the applicant is aware, the type of chrome ore used by him according to the invention has not been used commercially and therefore no published description, to the knowledge of applicant, has appeared elsewhere.

The expression "hybrid," used with reference to highly silicious low grade chrome ore, has been used by the applicant in an abbreviated sense to denote low grade chrome ore occurring in hybrid rocks, which latter have been formed by the intrusion of ultra-basic rock into ferruginous shale giving it a foliated (Schistose) appearance. The chrome ore grains occur as disseminations in this hybrid rock. The presence of high percentage of silica in the low grade chrome ore can be ascribed to chrome ore grains being intimately associated with shale and is therefore not capable of being separated out without expensive mechanical processing. The applicant aims at using this highly silicious chrome ore by employing chemical means.

Normally chrome ore in this region occurs mostly as pockets or veins in ultra-basic rocks. This normal chrome ore is of much higher grade than the low grade chrome ore referred to above.

The invention, therefore, resides in a process for the manufacture of refractory material from a low-grade non-refractory, highly silicious, hybrid chrome ore and consists in calcining such ore with amorphous magnesium oxide at a temperature corresponding to not less than Orton cone 26 (1595° C.) but preferably to cone 31 (1680° C.). During the process, the original structure of the hybrid chrome ore is completely altered with the formation of spinels and forsterite. The spinels formed are chrome spinel,  $\text{MgO}:\text{Cr}_2\text{O}_3$ ; magnesio ferrite,  $\text{MgO}:\text{Fe}_2\text{O}_3$ ; aluminum spinel,  $\text{MgO}:\text{Al}_2\text{O}_3$ . As a result of the process all of the silica in the original ore is converted into forsterite,  $2\text{MgO}:\text{SiO}_2$ .

The final product is therefore a mixture of the above-stated various spinels, forsterite and excess magnesium oxide in the form of the crystalline variety mineralogically known as periclase. All the formed minerals viz. spinels, forsterite and periclase have high melting points and hence, the end product made according to this invention has high refractoriness-under-load.

The formation of the crystalline phases of forsterite and spinels can take place only at high temperatures and in an oxidising atmosphere; as in the absence of oxygen, the undesirable fayalite ( $2\text{FeO}:\text{SiO}_2$ ) available in the composition may be formed from the ferrous oxide. Fayalite tends to reduce the (P. C. E.) of the mass. This can be avoided by converting the ferrous oxide ( $\text{FeO}$ ) to magnesioferrite  $\text{MgO}:\text{Fe}_2\text{O}_3$ .

Typical chemical analyses of chrome ores that fall within the scope of use according to this invention, as well as their pyrometric cone equivalents (fusion point) are given below:

### (a). Chemical analysis

|                         | (i)   | (ii)  | (iii) |
|-------------------------|-------|-------|-------|
| $\text{SiO}_2$          | 20.80 | 31.52 | 42.76 |
| $\text{Al}_2\text{O}_3$ | 7.50  | 8.00  | 7.12  |
| $\text{FeO}$            | 19.33 | 18.43 | 15.61 |
| $\text{CaO}$            | 0.60  | 0.30  | 0.20  |
| $\text{MgO}$            | 13.47 | 6.00  | 5.20  |
| $\text{Cr}_2\text{O}_3$ | 33.85 | 32.58 | 27.07 |
| Total Alkalies          | 0.50  | 0.30  | —     |
| Loss on Ignition        | 3.38  | 2.44  | 1.87  |

(b) *Pyrometric cone equivalent*  
(ORTON CONE)

Cone 20 (1530° C.) to 23 (1580° C.); 14 (1400° C.) to 16 (1465° C.); less than cone 14 (1400° C.).

According to the well known definition, a material to be classed as refractory should not have a P. C. E. of less than Orton cone 23. The above stated materials are, therefore, non-refractory and this invention confines itself only to the use of such non-refractory, highly silicious, hybrid chrome ores.

Moreover, if the equation of Schauer referred to above is applied to the typical analyses herein stated, the quotients would be much less than 1.38. These types of chrome ore according to Schauer are not suitable for the manufacture of refractories and, as is well known, they have been regarded as unsuitable also by the trade.

The source of magnesium oxide may be the naturally occurring mineral magnesite ( $MgCO_3$ ) or brucite ( $Mg(OH)_2$ ). The amorphous variety as distinct from the crystalline variety periclase has been experimentally found to be more suited to promote the chemical reactions for the production of spinels and forsterite as described hereinafter in greater detail. The nascent i. e. freshly formed amorphous magnesium oxide formed during heating together of the chrome ore and magnesite or brucite is found to give best results.

A special feature of the process is that no beneficiation of the ore is necessary for the removal of silica and other compounds which are commonly regarded as deleterious for making high grade refractories. On the other hand, these ingredients viz. silica, and iron compounds are valuable for the intended purpose as they yield, according to the specification herein described, valuable compounds with high melting points. Every unit of weight of the raw material used in this process therefore, goes into the finished product with the exception of the loss due to the removal of the slight amount of volatiles present, and the loss inherent in processing a material.

Referring now to the process in detail, highly silicious chrome ore and magnesite are separately ground, the degree of fineness of the latter being preferably more than that of the former. This, however, is not absolutely necessary if each ingredient is initially in a fine state of subdivision as described below. The chrome ore should be crushed and ground to pass through a screen whose openings are not larger than 4 mesh, Tyler screen (4.699 mm.). The magnesite, similarly should be crushed and ground to pass through a screen whose openings are not larger than 20 mesh, Tyler screen (0.833 mm.).

Although it has been stated that magnesite should be ground to a finer degree than the ore, it is clear that if the ore is already ground to pass through a 20 mesh screen, it is not necessary to grind the magnesite to a degree finer than to pass through a 20 mesh screen.

The two ground materials are then intimately mixed, preferably in a countercurrent mixer and heated in a kiln to a temperature corresponding to above Orton cone 26 (1595° C.) and, preferably, to Orton cone 31 (1680° C.).

During the heating, chemical reactions take place in the solid state which break down the original structure of the ore and form new components (spinels and forsterite), with high melting points, as follows:

(a)  $SiO_2$  of the ore combines with  $MgO$  to form forsterite according to the equation



(forsterite).

(b) and similarly  $Al_2O_3 + MgO = MgO:Al_2O_3$  (aluminous spinel).

(c)  $2FeO + O + MgO = MgO:Fe_2O_3$  (the spinel, magnesiaferrite).

(d)  $Cr_2O_3 + MgO = MgO:Cr_2O_3$  (chrome spinel).

From the chemical equations given above, it is possible to readily determine the weights of  $MgO$  or ( $MgCO_3$ )

required for one part by weight of each of the ingredients,  $SiO_2$ ;  $Al_2O_3$ ;  $FeO$ ; and  $Cr_2O_3$ , present in the original ore.  $MgO$  by weight, required for one part by weight of each of the above is: 1.3; 0.4; 0.27; and 0.24 respectively.

5 It follows that for a chrome ore having a composition corresponding to sample analysis (II) above, the minimum requirement of  $MgO$  would be:  $(31.52 \times 1.3) + (8 \times 0.4) + (18.43 \times 0.27) + (32.58 \times 0.24) = 56.92$  (or equivalent of 121.8 parts of  $MgCO_3$ ) i. e. 1 part of chrome ore would require 0.57 part of  $MgO$  or 1.21 parts of  $MgCO_3$ .

In the above calculation, the percent of  $MgO$  available in the chrome ore has been neglected. As a matter of fact, addition of an excess  $MgO$  (or  $MgCO_3$ ) is preferable, since  $MgO$  is converted to periclase in the final product and thereby adds to the desirable physical properties of the final composition.

It has been found that when magnesite ( $MgCO_3$ ) is employed, best results are obtained when 50% more than the theoretically required amount of magnesite is used. Thus, instead of using 1.21 parts of  $MgCO_3$  for every part of chrome ore, it is preferred to use 1.8 parts of  $MgCO_3$ .

The proportion of required magnesite with respect to chrome ore is determined by the exact percentages of the various oxides present in the chrome ore. The permissible range is 1 part ore to 0.75-2.0 parts magnesite, the parts being by weight. If magnesium oxide is employed, then the proportion of chrome ore to magnesium oxide is 1 to 0.375-1.0 by weight.

The  $MgCO_3$  referred to in the above calculations had the following approximate chemical analysis:

| Silica | $Fe_2O_3$ | $CaO$ | $MgO$ | loss  |
|--------|-----------|-------|-------|-------|
| 1.16   | 0.20      | 1.00  | 46.70 | 50.70 |

35 The mass, after heating or calcining in a kiln, is crushed and sieved through different mesh sieves. Different proportions of sieved material are blended together without further crushing, mixed with an organic binder such as molasses or sulphite lye or lightly calcined magnesite and moulded into bricks or like shapes. These bricks may be used as such or after they have been fired in a kiln. For extreme severe conditions of service a second firing is preferred and this should be done at a temperature not less than Orton cone 18 (1490° C.) and preferably at Orton cone 30 (1650° C.).

40 According to a modification of the process, in order to lower the temperature of conversion to forsterite and spinels, fluxes such as boric acid and volatile salts such as ammonium sulphate or ammonium chloride may be added to the mixed mass prior to calcination, the fluxes being not less than 1.5 per cent but not more than 2 per cent of the total weight of the mass. The temperature of calcination of the mass with fluxes should not be less than Orton cone 20 (1530° C.). The boric acid, although aiding conversion, lowers the refractoriness-under-load value.

45 Tests on a few typical samples, compositions of which are given earlier in the specifications show that the final product has the following superior physical properties:

50 (I) *Refractoriness-under-load*.—A refractory made according to this process, when tested under a load of 2 kg./cm.<sup>2</sup> did not deform at 1700° C. whereas most commercial grades of brick made from high grade chrome ore and magnesite, under the same load deformed at 1570° C. and completely collapsed at 1650° C.

55 (II) *Resistance against attack of iron oxide*.—A 3" x 2" x 2" piece of refractory made according to this invention, when heated with a layer of 100 gram mill scale at 1600° C., and soaked for one hour at this temperature showed "Bursting Expansion" of 2%, as against

6 to 16% for commercial grades of brick made from high grade chrome ore and magnesite.

(III) *A. S. T. M. load test at 1450° C.*—On subjecting bricks made by the process of the present invention to A. S. T. M. load test at 1450° C., it was found that the brick gave a contraction of 0.48% whereas commercial grades of brick failed by shearing diagonally at 1420° C.

Although the present invention has been shown and described in specific embodiments, nevertheless, various changes and modifications obvious to one skilled in the art are within the spirit, scope, and contemplation of the invention.

What is claimed is:

A novel refractory material having a high pyrometric cone equivalent and high refractoriness-under-load prepared by mixing together one part by weight of chrome ore containing about 20% to 43% by weight of  $\text{SiO}_2$ ,

about 5% to about 13% by weight of  $\text{MgO}$ , about 22% to 27% by weight of  $\text{FeO}$  and  $\text{Al}_2\text{O}_3$  combined, and about 27% to 34% by weight of  $\text{Cr}_2\text{O}_3$  and characterized by a pyrometric cone equivalent below the temperature corresponding to Orton cone 23 and from about 0.375 to about 1.0 part by weight of amorphous magnesium oxide, both in a state of fine subdivision, the mixture being calcined at a temperature from about Orton cone 26 (1595° C.) to about Orton cone 31 (1680° C.) such that new compounds are formed.

**References Cited in the file of this patent**

**FOREIGN PATENTS**

|    |         |               |       |      |
|----|---------|---------------|-------|------|
| 15 | 631,010 | Germany       | ----- | 1936 |
|    | 435,448 | Great Britain | ----- | 1935 |
| 10 | 146,725 | Australia     | ----- | 1949 |